

1

3,041,326

**SOLUBILIZED DERIVATIVES OF ROSINS AND  
PROCESS OF SOLUBILIZATION**

Charles V. Wilson and William J. Knox, Jr., Rochester,  
N.Y., assignors to Eastman Kodak Company, Rochester,  
N.Y., a corporation of New Jersey  
No Drawing. Filed Aug. 9, 1956, Ser. No. 603,195  
11 Claims. (Cl. 260—97)

This invention relates to new compositions of matter obtained from commercial rosin and to the use of these products, more particularly, their use as detergents and as coating aids.

Rosin is a relatively inexpensive, commercially available material widely used for various purposes, as such, and in several modifications, for example those produced by hydrogenation or dehydrogenation. Rosin acids are useful surface-active agents particularly in combination with fatty soaps to impart increased solubility and foaming power. However, rosin soaps tend to discolor on aging and, like the fatty acid soaps, they are not resistant to lime and acids.

In order to avoid discoloration, rosin is modified commercially by hydrogenation or dehydrogenation. The former process eliminates the double bonds, while the latter partially aromatizes the compounds. In either case, the resulting products are less susceptible to oxidative deterioration. These hydrogenated or dehydrogenated rosins are used to increase the efficiency of soaps both for laundry and toilet purposes.

These treatments, however, do not make the materials lime resistant nor do they increase the solubility substantially. One of the components of rosin, laevo-pimaric acid is made more soluble by reacting with maleic anhydride and hydrolyzing the maleopimaric acid thus formed to the sodium salt. However, laevo-pimaric acid makes up only 10 to 15% of the rosin, and it has been considered desirable to solubilize all the rosin acids in the mixture. We have found that the solubility of these complex molecules may be improved and that in several cases the products have a high degree of calcium tolerance.

We have also found that many of these materials have detergent properties which permit their use as wetting agents and coating aids.

There are many instances in industry where it is desirable to apply one or more relatively thin coatings or layers to various type bases. In the photographic industry particularly, products are prepared by applying relatively thin coatings to various types of bases such as film and paper bases. It is usually preferable that these coatings be uniform and that the coated base be free of bare spots or other imperfections. It is also desirable to apply such coatings at good production speeds for efficiency of operation.

In the coating of photographic film or paper with a gelatin layer such as a photographic emulsion or other coating compositions, a uniform coating must be obtained. In the absence of a coating aid, numerous small crescent-shaped uncoated areas are observed in the final product. These defects may be the size of a pin head with streaks running from the points of the crescent in a direction opposite to that of coating. Sometimes lightly coated areas from 5 to 10 mm. in diameter may also appear.

Various surface-active agents have been employed in gelatin coating compositions for facilitating coating procedures or operations. For instance, saponin has been used for this purpose and eliminates many of the defects in coatings, giving a uniformly even coating particularly where the gelatin layer is applied to a dry surface.

2

Saponin, however, is a naturally occurring material of vegetable origin and may vary markedly from batch to batch in quality as well as composition. The quality of some batches of saponin may cause an increase in fog or a decrease of sensitivity of certain emulsions or may even result in no improvement in the coating properties of the composition to which it is added. These wide variations in the quality of this natural material make preferable, as coating aids, surface-active agents which are reproducible from batch to batch both in chemical composition and coating behavior.

A number of synthetic agents have utility for coating purposes, but they are often deficient in some respects. For example, certain coating aids naturally contribute to the ease of coating, but they are not useful because of adverse photographic properties. Various other difficulties and problems arise in the photographic industry in the application of gelatin layers to a support.

One object of this invention is to solubilize complex molecules such as rosin, rosin acids, and the like. Another object of this invention is to provide highly water-soluble rosin derivatives which have a high degree of calcium tolerance. An additional object is to provide a coating aid free from photographic activity for coating photographic emulsions. Another object is to provide a method for applying gelatin coatings in the preparation of photographic materials which are uniformly even and repellency free and which are photographically inert. A further object of our invention is to prepare wetting agents which may be used as detergents. Other objects will appear herein.

We have found that ordinary rosin, laevo-pimaric acid, the mixture of rosin acids remaining after removal of the laevo-pimaric acid, and related products will react with isocyanate esters, particularly those derived from aspartic and glutamic acids. The resulting materials can be selectively hydrolyzed to the sodium salts of acids which are highly water soluble and have a high degree of calcium tolerance. The reaction with the abietic acid portion of the mixture (and the others react similarly) may be represented as follows:



In the above reaction sequence, R represents a simple alkyl radical such as methyl or ethyl, and n is a whole integer from 1 to 3.

The products are quite dark in color, but the hydrogenated and dehydrogenated materials which are available commercially react in exactly the same manner and give lighter colored products. These hydrogenated and dehydrogenated materials are also intended herein in referring to rosins, etc.

Maleopimamic acid reacted with isocyanato esters and selectively hydrolyzed, yields products having the following general structure:



in which R may be H, CH<sub>3</sub>, C<sub>2</sub>H<sub>5</sub>, —CH(CH<sub>3</sub>)<sub>2</sub>, C<sub>6</sub>H<sub>5</sub> or —(CH<sub>2</sub>)<sub>n</sub>COONa where n=1 to 3. These products are hereinafter referred to as sodium salts of maleopimaro-yl-amino acids. Thus, for example, if R is CH<sub>3</sub>, the product is trisodium maleopimaro-ylglycinate, while if R is —CH<sub>2</sub>COONa, the product is tetrasodium maleopimaro-ylaspartate.

Other products derived from rosin, for example, Abitol and Rosin Amine D and various hydrogenated and dehydrogenated forms of the mixture of alcohols or amines, as well as their polyoxyethylene derivatives also react with isocyanato esters to produce urethanes and ureas respectively.

Rosin Amine D is the trade name for a commercially available material which is essentially 1-aminomethyl-7-isopropyl-1,4a-dimethyl-1,2,3,4a,9,10,10a-octahydrophenanthrene.

Abitol and the products derived from it by treatment with ethylene oxide are particularly useful because further treatment with any of a number of isocyanato esters produces, after selective hydrolysis, products of high water solubility and a high degree of calcium tolerance. Substances of this type are available on the market under the trade names "Synthetics AD-50," "Synthetics AD-150" and "Synthetics AD-400." "Abitol" comprises a mixture of the three alcohols having about 15% of non-alcoholic material and corresponding ratios of 45% tetrahydroabietyl alcohol, 15% dehydroabietyl alcohol, and 40% dehydroabietyl alcohol having the following structures:



The 15% comprising the average non-alcohol portion of Abitol contains approximately 3-8% ester which can be considered as methyl esters of hydrogenated rosin; the remainder about 7-12%, is similar to the hydrocarbon fractions occurring in hydrogenated rosin.

The derivatives of "Abitol" formed by treatment with ethylene oxide may be represented as a mixture of the following three structures:



5 n may be 1-10 but in our preferred embodiment, n is 3 to 6. Synthetics AD-50 represents a derivative of Abitol with ethylene oxide in which n is about 5.4.

The materials described in the following examples as sodium rosinyl glutamate and sodium rosinyl aspartate are amides which were obtained by reacting a mixture of rosin acids with dimethyl isocyanatoglutamate or succinate. The term "rosinyl" is used here to signify the acyl radicals of the mixture of rosin acids present in commercial rosin. Tetra-sodium maleopimaro-ylglutamate and aspartate are

55 also amides prepared by reacting maleopimamic acid with the appropriate isocyanato ester and selectively hydrolyzing the primarily formed amide-ester. The Rosin Amine D derivative referred to in Example 12 is a urea prepared by reacting Rosin Amine D with the isocyanato ester.

60 The last three materials in Examples 13-16 are urethanes obtained by the reaction of the isosyanato ester with a rosin alcohol known as "Abitol" or polyethoxy derivative thereof.

The following examples illustrate our invention but are not to be construed as limiting it in any way.

### EXAMPLE 1

#### Sodium Rosinylaspartate

70 A mixture of 60 parts of a commercial rosin, 39 parts (somewhat less than one molar equivalent based on abietic acid) of diethyl isocyanatosuccinate, and 50 parts of dry chlorobenzene was heated for 16-18 hours near the boiling point of the solvent (130-140°). There was 75 evolution of carbon dioxide during the first few hours of

the reaction. The solvent was removed under reduced pressure, and the residue (95 parts) dissolved in 400 parts of alcohol and filtered. To the alcohol solution at 33° was added a solution of 15 parts of sodium hydroxide in 15 parts of water and 150 parts of alcohol. Precipitation of a solid began shortly after mixing, and the temperature rose to about 45°. The solid tends to form a gum if heated above this temperature so the mixture was allowed to stand for several hours to insure complete hydrolysis of the ester groups. The resulting sodium salt was collected on a filter, washed with acetone, and dried. The yield was about 30 parts.

Removal of solvent from the filtrate, using benzene to azeotrope off the last of the water, left 52 parts of a darker solid than that described above.

Both solids are very soluble in water, have a high calcium tolerance, and are active surface-active agents.

Since commercial rosin is a mixture of several related acids, the reaction is best represented as follows:



### EXAMPLE 2

#### Tetrasodium Maleopimaroylaspartate

A solution of 40 grams (0.1 m.) of maleopimaric acid (obtained from gum oleoresin by treatment with maleic anhydride as described in U.S. Patent 2,359,980) and 21.5 g. (0.1 m.) of diethylisocyanato succinate in 60 ml. of chlorobenzene was heated for 16-18 hours at the boiling point. Carbon dioxide was evolved during the early stages of the reaction. The solvent was removed by heating on the steam bath under reduced pressure, and the residue was dissolved in 300 ml. of alcohol. Treatment of this solution with a solution of 16 g. (0.4 m.) of sodium hydroxide in aqueous alcohol (made by dissolving the sodium hydroxide in 20 ml. of water and diluting with 200 ml. of alcohol) caused precipitation of a gummy solid. The mixture was heated for an hour at 65°, allowed to come to room temperature, and the aqueous alcohol removed by decantation. Acetone was added and the solid ground to a powder by use of a mortar and pestle, or alternately, by vigorous stirring with a Lightnin' mixer. The solid was collected on a filter, washed with acetone and dried. The yield of product was 55-60 g. It had high water solubility, excellent calcium tolerance, and good surface-active properties.

A similar product, tetrasodium maleopimaroylglycinate, results by treatment of maleopimaric acid with dimethyl isocyanatoglutarate by the same procedure. Similar products may be obtained by using isocyanato esters such as those derived from glycine,  $\alpha$ -alanine, leucine and the like.

### EXAMPLE 3

#### Urea From Rosin Amine D (Hercules) and Dimethyl Isocyanato Succinate

Dimethyl isocyanato succinate (23.5 g.) was added to 36 g. (1 molar equivalent) of Rosin Amine D. There was considerable heat of reaction, the temperature rising to 70-80°. The mixture was heated for several hours at 90-100°. On cooling it set to a resin-like mass. It was dissolved in alcohol and treated with 10 g. of sodium hydroxide dissolved in 12 ml. of water, and diluted with alcohol. There was a small temperature rise; hydrolysis was completed by heating for 1-2 hours at 65°. The sodium salt which separates in resinous form became solid on cooling. The aqueous alcohol was removed by decantation, and a mixture of acetone and ethyl acetate added. After standing overnight, the solid was broken up, collected on a filter, washed with acetone, dried,

powdered, slurred with acetone, refiltered, and dried. The product (52 g.) was soluble in water but not tolerant of calcium. It was essentially N- $\alpha$ , $\beta$ -dicarboxyethyl-N'-(7 isopropyl-1,4a-dimethyl)-1,2,3,4,4a,9,10,10a-octahydrophenanthrylmethylurea (disodium salt).

### EXAMPLE 4

#### Sodium N-Carbo "Abity" Oxyglutamate<sup>1</sup>

A mixture of 544 g. (1.88 m.) of Abitol (Hercules) and 384 g. (1.91 m.) of dimethyl isocyanatoglutarate was heated at 130° for two hours. The resulting product was dissolved in 1500 ml. of ethanol and treated while being stirred with 160 g. of sodium hydroxide in 175 ml. of water. After the addition of the alkali, the mixture was heated at 75° for an hour, cooled, and the solid collected on a filter, washed with alcohol, and dried. There was obtained about 750 g. of granular product which has high solubility and good calcium tolerance. The material was an excellent surface-active agent and a good coating assistant.

### EXAMPLE 5

#### N-Carbo "Abity" Oxypolyethoxyglycine (Na Salt)

A mixture of 75 g. of Synthetics AD-50, a derivative of Abitol (see Example 4) with ethylene oxide, and 26 g. of ethyl isocyanatoacetate reacted exothermically. When the primary reaction was over, the mixture was heated at 70-80° for 5-6 hours, and the product dissolved in 300 ml. of alcohol. To the alcoholic solution was added 10 g. of sodium hydroxide in 12 ml. of water. The mixture was heated at 65-70° for about one-half hour and then allowed to stand for several hours. A small amount of solid that separated in the solution was removed by filtration; it was the disubstituted urea formed from the ethyl isocyanatoacetate. The water and alcohol were removed from the filtrate under reduced pressure to give 88 g. of a syrup which could be dissolved in water to give a solution of any desired strength. Alternatively, the hydrolysis can be carried out with water and the aqueous solution thus formed adjusted to the desired strength. Sodium N-carboabityloxypolyethoxyglutamate can be prepared by a similar procedure.

<sup>1</sup> Abitol is essentially a mixture of three alcohols of the following structures:



The name given to the product of this example is chosen to indicate that said product is a mixture of the urethanes of these three alcohols.

7  
EXAMPLE 6

In an air knife application to paper of a silver bromide emulsion involving the use of sodium "rosinyl" glutamate (SRG) as a coating aid, the following results were obtained:

| Coating Aid | Concentration, grams per pound | Repellencies per 7.5 ft. sq. | Photographic Properties |
|-------------|--------------------------------|------------------------------|-------------------------|
| Blank       | 0.0                            | 1                            | Satisfactory.           |
| SRG         | 0.13                           | 5                            | Do.                     |
| Do          | 0.25                           | 1                            | Do.                     |
| Do          | 0.5                            | 0                            | Do.                     |
| Do          | 1.0                            | 2                            | Do.                     |

## EXAMPLE 7

In an experiment similar to that described in Example 6, but involving sodium "rosinyl" aspartate (SRA), the following results were obtained:

| Coating Aid | Concentration, grams per pound | Repellencies per 7.5 ft. sq. | Photographic Properties |
|-------------|--------------------------------|------------------------------|-------------------------|
| Blank       | 0.0                            | 3                            | Satisfactory.           |
| SRA         | 0.13                           | 0                            | Do.                     |
| Do          | 0.25                           | 1                            | Do.                     |
| Do          | 0.5                            | 0                            | Do.                     |
| Do          | 1.0                            | 2                            | Do.                     |

## EXAMPLE 8

In an experiment similar to that described in Example 6, but involving tetra-sodium maleopimaroylglutamate (SMG) as a coating aid, the following results were obtained:

| Coating Aid | Concentration, grams per pound | Repellencies per 7.5 ft. sq. | Photographic Properties |
|-------------|--------------------------------|------------------------------|-------------------------|
| Blank       | 0.0                            | 6                            | Satisfactory.           |
| SMG         | 0.13                           | 1                            | Do.                     |
| Do          | 0.25                           | 0                            | Do.                     |
| Do          | 0.5                            | 0                            | Do.                     |
| Do          | 1.0                            | 0                            | Do.                     |

## EXAMPLE 9

In an experiment similar to that described in Example 6, but involving tetra-sodium maleopimaroylaspartate (SMA) as a coating aid, the following results were obtained:

| Coating Aid | Concentration, grams per pound | Repellencies per 7.5 ft. sq. | Photographic Properties |
|-------------|--------------------------------|------------------------------|-------------------------|
| Blank       | 0.0                            | 3                            | Satisfactory.           |
| SMA         | 0.13                           | 0                            | Do.                     |
| Do          | 0.25                           | 0                            | Do.                     |
| Do          | 0.5                            | 0                            | Do.                     |
| Do          | 1.0                            | 0                            | Do.                     |

## EXAMPLE 10

In an experiment similar to that described in Example 6, but involving the Rosin Amine D Derivative (RDA) as a coating aid, the following results were obtained:

| Coating Aid | Concentration, grams per pound | Repellencies per 7.5 ft. sq. | Photographic Properties |
|-------------|--------------------------------|------------------------------|-------------------------|
| Blank       | 0.0                            | 3                            | Satisfactory.           |
| RDA         | 0.13                           | 3                            | Do.                     |
| Do          | 0.25                           | 1                            | Do.                     |
| Do          | 0.5                            | 1                            | Do.                     |
| Do          | 1.0                            | 1                            | Do.                     |

## EXAMPLE 11

In an experiment similar to that described in Example 6, but involving the product of Example 4, sodium N-

7  
8  
carboabityloxyglutamate (SCG), as a coating aid, the following results were obtained:

| Coating Aid | Concentration, grams per pound | Repellencies per 7.5 ft. sq. | Photographic Properties |
|-------------|--------------------------------|------------------------------|-------------------------|
| Blank       | 0.0                            | 10                           | Satisfactory.           |
| SCG         | 0.13                           | 10                           | Do.                     |
| Do          | 0.25                           | 2                            | Do.                     |
| Do          | 0.5                            | 0                            | Do.                     |
| Do          | 1.0                            | 0                            | Do.                     |

## EXAMPLE 12

In an experiment similar to that described in Example 6, but involving sodium N-carboabityloxyglycinate (SAG) as a coating aid, the following results were obtained:

| Coating Aid | Concentration, grams per pound | Repellencies per 7.5 ft. sq. | Photographic Properties |
|-------------|--------------------------------|------------------------------|-------------------------|
| Blank       | 0.0                            | 6                            | Satisfactory.           |
| SAG         | 0.13                           | 0                            | Do.                     |
| Do          | 0.25                           | 0                            | Do.                     |
| Do          | 0.5                            | 0                            | Do.                     |
| Do          | 1.0                            | 3                            | Do.                     |

## EXAMPLE 13

In an experiment similar to that described in Example 6, but involving a product as described in Example 5, sodium N-carboabityloxypolyethoxy glutamate (SCPG), the following results were obtained:

| Coating Aid | Concentration, grams per pound | Repellencies per 7.5 ft. sq. | Photographic Properties |
|-------------|--------------------------------|------------------------------|-------------------------|
| Blank       | 0.0                            | 7                            | Satisfactory.           |
| SCPG        | 0.13                           | 8                            | Do.                     |
| Do          | 0.25                           | 0                            | Do.                     |
| Do          | 0.5                            | 1                            | Do.                     |
| Do          | 1.0                            | 0                            | Do.                     |

## EXAMPLE 14

In an experimental pellloid coating obtained by using the slide hopper coating technique described in U.S. Patent No. 2,681,294 and involving the product of Example 4, sodium N-carboabityloxyglutamate (SCG), at 0.22 gm./lb. of coating melt as a coating aid, the following results were obtained:

|       | Repellencies, 25 ft. sq. | Mottle       | Streakiness | Nature of Dried Surface |
|-------|--------------------------|--------------|-------------|-------------------------|
| Blank | 4                        | sl. to sl. + | sl.         | Rough.                  |
| SCG   | 0                        | sl.          | sl.         | Do.                     |

## EXAMPLE 15

In an experiment similar to that described in Example 14, but involving the product of Example 5, sodium N-carboabityloxyglycinate (SAPG), as a coating aid, the following results were obtained:

|       | Repellencies, 25 ft. sq. | Mottle | Streakiness | Nature of Dried Surface |
|-------|--------------------------|--------|-------------|-------------------------|
| Blank | 10                       | Med.   | sl.         | Rough.                  |
| SAPG  | 2                        | sl.    | sl.         | Do.                     |

## EXAMPLE 16

In an experiment similar to that described in Example 14, but involving the product mentioned in Example 5,

sodium N-carboabityloxypolyethoxyglutamate (SCPG), the following results were obtained:

|       | Repellencies, 25 ft. sq. | Mottle | Streakiness | Nature of Dried Surface |
|-------|--------------------------|--------|-------------|-------------------------|
| Blank | 13                       | sl.    | sl.         |                         |
| SCPG  | 2                        | sl.    | sl.         |                         |

## EXAMPLE 17

In an X-ray emulsion coating trial in which a product as described in Example 5, sodium N-carboabityloxypolyethoxyglutamate was used, the ease of the wet-on-wet coating was essentially equivalent to that obtained with oleoylpolyptide, an excellent wet-on-wet coating aid derived from hydrolyzed gelatin and oleoyl chloride, which is used as a standard of coating excellence. The photographic properties of this material are very satisfactory in many emulsion systems. The ratio by weight of coating aid to coating melt was 0.1 gram to 2.5 pounds in the emulsion and 0.1 gram to 7.7 pounds in the overcoat.

## EXAMPLE 18

In runs similar to those in Example 17 but using the product of Example 5, sodium N-carboabityloxypolyethoxy glycinate, at concentrations of 1.0 gram to 2.5 pounds of wet emulsion and 1 gram to 7.7 pounds of overcoat melt, comparably good results were obtained.

Examples 17 and 18 are wet-on-wet coating examples where a warm overcoat is applied to a wet emulsion surface which has been set by chilling.

The term "rosinyl" has been applied to the 19 carbon alkylated hydrophenanthrene nucleus which occurs in the rosin acids and the partially hydrogenated rosin acids. "Rosinyl" is thus well known as the generic name of the  $C_{19}H_{29}$  and  $C_{19}H_{31}$  radicals which occur in abietic acid, levopimamic acid, neoabietic acid, dextropimamic acid and like acids whose general formula is  $C_{19}H_{29}COOH$ , and dihydroabietic acid, dihydrolevopimamic acid, dihydrodextropimamic acid and like acids whose general formula is  $C_{19}H_{31}COOH$ . The term "rosinyl" is likewise here applied broadly to the  $C_{19}H_{29}$  and the  $C_{19}H_{31}$  radicals which occur in the rosin acids and the dihydrorosin acids. The term "hydrorosinyl" refers to the  $C_{19}H_{33}$  radical having the ring structure of the fully hydrogenated rosin acids, and the term "dehydrorosinyl" refers to the  $C_{19}H_{27}$  radical having the ring structure of dehydroabietic acid. The terms norabietyl, nordihydroabietyl, nortetrahydroabietyl, and nordehydroabietyl are the specific names applied to those radicals which have the ring structure of abietic acid, dihydroabietic acid, tetrahydroabietic acid and dehydroabietic acid respectively wherein the point of linkage is carbon number one.

When the compositions disclosed herein are used as coating aids, the aid may be incorporated in a gelatin coating which is coated on various supports such as paper, film base, glass and the like. In addition, some of these materials may be used for coatings over wet surfaces as well as dry surfaces. For instance, they may be used as coating aids when a gelatin emulsion is coated over a previous gelatin emulsion which is still in a wet condition such as a wet chilled emulsion surface. Moreover, some of these coating aids may be used in a series of gelatin layers and the subsequent gelatin layer containing one of these coating aids may be coated over a wet chilled emulsion surface, in which wet chilled emulsion has been incorporated one of these coating aids. Other combinations of layers in wet or dry condition and in various sequences in which one or more layers contain one of these coating aids are intended to be within the scope of our invention.

Water-soluble salts other than the sodium salts are also within the scope of this invention and may be formed by using the appropriate hydroxide such as potassium hy-

dioxide, ammonium hydroxide and the like to hydrolyze the ester.

These coating aids are also advantageous with a multiple layer coating technique of the type described in U.S. patent application Serial No. 489,863, now U.S. Patent No. 2,761,791.

We claim:

1. A composition of matter having the following formula:

10



15

in which R is the carbocyclic nucleus of a rosin acid selected from the class consisting of rosinyl, hydrorosinyl and dehydrorosinyl radicals, in which n is 0-1 and when n is 1, X is  $CH_2NH$ , R' is selected from the class consisting of alkyl radicals having 1-4 carbon atoms, hydrogen, phenyl,  $COOR''$ ,  $CH_2COOR''$ ,  $(CH_2)_2COOR''$ , and  $(CH_2)_3COOR''$ , and R'' is an alkyl group having 1-3 carbon atoms.

20

2. A composition of matter having the following formula:



25

in which R is selected from the class consisting of H, alkyl with 1-4 carbon atoms, phenyl,  $COONa$ ,  $CH_2COONa$ ,  $CH_2CH_2COONa$ , and  $(CH_2)_2COONa$ .

30

3. A composition of matter having the following formula:

40



45

45

50

50

55

55

60

60

65

65

70

70

75



in which R is a rosinyl nucleus.

5. A composition of matter comprising a mixture of the following structures:





in which the structures are represented in the mixture in the amounts of 45%, 15%, and 40%.

6. A process of solubilizing a complex molecule by reacting an isocyanato ester having the following general formula:



in which R is an alkyl group having 1-3 carbon atoms and R' is selected from the class consisting of H, phenyl, alkyl with 1-4 carbon atoms, COOR, CH<sub>2</sub>COOR,



and (CH<sub>2</sub>)<sub>3</sub>COOR in which R is an alkyl group having 1-3 carbon atoms, with a material selected from the class consisting of rosin, rosin acids, 1-amino-methyl-7-isopropyl - 1,4a - dimethyl - 1,2,3,4,4a,9,10,10a - octahydrophenanthrene, rosin alcohols, hydrogenated rosin acids and dehydrogenated rosin acids and hydrolyzing the ester linkage with alkali.

7. A process of improving the solubility of rosin acids comprising reacting a mixture consisting essentially of rosin acids with an isocyanato ester having the following general formula:



in which R is an alkyl group having 1-3 carbon atoms and R' is selected from the class consisting of H, phenyl, alkyl with 1-4 carbon atoms, COOR, CH<sub>2</sub>COOR,



and (CH<sub>2</sub>)<sub>3</sub>COOR and hydrolyzing the ester linkage with alkali.

8. A process of improving the solubility of hydrogenated rosin acids comprising reacting a mixture consisting essentially of hydrogenated rosin acids with an isocyanato ester having the following general formula:



in which R is an alkyl group having 1-3 carbon atoms and R' is selected from the class consisting of H, phenyl, alkyl with 1-4 carbon atoms, COOR, CH<sub>2</sub>COOR,



and (CH<sub>2</sub>)<sub>3</sub>COOR and hydrolyzing the ester linkage with alkali.

9. A process of improving the solubility of rosin alco-

hols comprising reacting a mixture consisting essentially of rosin alcohols with an isocyanato ester having the following general formula:



in which R is an alkyl group having 1-3 carbon atoms, and R' is selected from the class consisting of H, phenyl, alkyl with 1-4 carbon atoms, COOR, CH<sub>2</sub>COOR, (CH<sub>2</sub>)<sub>2</sub>COOR, and (CH<sub>2</sub>)<sub>3</sub>COOR and hydrolyzing the ester linkage with alkali.

10. A process of improving the solubility of dehydrogenated rosin acids comprising reacting a mixture consisting essentially of dehydrogenated rosin acids with an isocyanato ester having the following general formula:



in which R is an alkyl group having 1-3 carbon atoms, and R' is selected from the class consisting of H, phenyl, alkyl with 1-4 carbon atoms, COOR, CH<sub>2</sub>COOR, (CH<sub>2</sub>)<sub>2</sub>COOR, and (CH<sub>2</sub>)<sub>3</sub>COOR and hydrolyzing the ester linkage with alkali.

11. A process of improving the solubility of polyoxyethylene derivatives of rosin alcohols which are formed by reacting rosin alcohols with ethylene oxide comprising reacting a mixture consisting essentially of polyoxyethylene derivatives of rosin alcohols with an isocyanato ester having the following general formula:



in which R is an alkyl group having 1-3 carbon atoms, and R' is selected from the class consisting of H, phenyl, alkyl with 1-4 carbon atoms, COOR, CH<sub>2</sub>COOR, (CH<sub>2</sub>)<sub>2</sub>COOR, and (CH<sub>2</sub>)<sub>3</sub>COOR and hydrolyzing the ester linkage with alkali.

#### References Cited in the file of this patent

##### UNITED STATES PATENTS

|    |           |                  |               |
|----|-----------|------------------|---------------|
| 40 | 2,035,024 | Schur            | Mar. 24, 1936 |
|    | 2,354,662 | Bryce            | Aug. 1, 1944  |
|    | 2,472,437 | Pratt            | June 7, 1949  |
|    | 2,499,430 | Vogel et al.     | Mar. 7, 1950  |
| 45 | 2,750,365 | Subluskey        | June 12, 1956 |
|    | 2,875,214 | Humphlett et al. | Feb. 24, 1959 |

##### FOREIGN PATENTS

|    |           |         |                |
|----|-----------|---------|----------------|
| 50 | 676,511   | Germany | June 8, 1939   |
|    | 1,037,362 | France  | Sept. 16, 1953 |

##### OTHER REFERENCES

Brewster: Organic Chemistry, page 228, Prentice-Hall (1948).

Pinner: Plastics, vol. 11, pages 206-11; 215; 257 (1947). Staff Report, Paint, Oil and Chemical Review, vol. 116, pages 28-30, No. 26 (1953).